

# UNITED STATES PATENT OFFICE.

ROBERT MACPHERSON, OF BRONDESURY, AND WILLIAM EDWIN HEYS, OF BUSHEY,  
ENGLAND.

## DETERGENT FOR USE WITH HARD AND SALT WATERS.

No. 902,750.

Specification of Letters Patent.

Patented Nov. 3, 1908.

Application filed February 10, 1906. Serial No. 300,467.

*To all whom it may concern:*

Be it known that I, ROBERT MACPHERSON, a resident of Brondesbury, in the county of Middlesex, England, and WILLIAM EDWIN HEYS, a resident of Bushey, in the county of Hertford, England, both subjects of the King of Great Britain and Ireland, have invented a new or Improved Detergent for use with Hard and Salt Waters, of which the following is a specification.

This invention relates to a new detergent by means of which clothing, linen, textile materials and fabrics, paint, woodwork and the like may be washed or cleansed in sea-water and other hard waters.

"Marine soaps" are already known and used for the purposes above set forth, and have as their basis saponified cocoa-nut oil, but such soaps are open to objections which are entirely removed or obviated by means of this new detergent. For example, the known marine soaps leave a very permanent and objectionable odor in the linen and other articles washed therewith; it is very difficult to remove from the goods the lime and the magnesia soaps which are formed during the washing by sea-water and which are practically insoluble in water; the soaps are soluble with great difficulty and only to a limited extent so that their efficiency is low while their cost is high. On the other hand the new detergent, made as herein-after indicated, leaves no permanent odor; the slight amount of insoluble soap produced is readily removed by rinsing; it dissolves with great facility in sea and hard waters; and its cost is lower.

The materials which we employ in the manufacture of the new detergent are:—  
40 cocoa-nut oil or cocoa-nut olein or an analogous oil or olein from which a soap soluble in sea water can be produced, known as "cocoa-nut olein"; a suitable vegetable proteid substantially free from fatty acids other than that or those which are contained or are analogous with that or those contained in cocoa-nut oil and are similarly capable of producing a "lather" in sea-water when saponified; a soda or potash lye 50 of higher strength than is used in ordinary soap manufacture; water when necessary; and, optionally, farina and other "fillers."

In carrying the process of manufacturing the new detergent into effect the proteid matter is so treated with a sufficiency of

strong alkali under heat that it is broken down and the thereby disassociated amino-fatty acids are saponified by the alkali together with the cocoanut olein.

The "cocoa-nut olein" may be mixed with the proteid matters and heated to upwards of 100° C. 120° or 130° give advantageous results with stirring. After a short time the lye is added with continued stirring while the temperature is maintained at from 80° C. to 90° C. Saponification takes place rapidly, and the resulting mass when cool can be granulated by being passed through sieves, after which it may be reduced to powder in a disintegrator. It is convenient to add the farina or other "filler" to the oil with the proteid matter, so as to avoid the cooling effect which their subsequent addition would produce. Alternatively, the "cocoa-nut olein" may first be separately heated to above 100° C., and the proteid may be added to the hot oil before saponification, or immediately after the addition of the lye, or the proteid matters may be separately acted on with the whole or part of the lye and the "cocoa-nut olein" be then added thereto with subsequent addition of the remainder of the lye, if any. Sufficient heat must be employed in the process to insure the coagulation of albuminous and mucilaginous matters contained in the "cocoa-nut olein" and in the proteid matters and for the formation of amido fatty acids from the proteid under the action of the lye, as is indicated by the evolution of ammonium carbonate fumes.

An excess of lye beyond that necessary for the saponification of the "cocoa-nut olein" is necessary to be used so as to insure the saponification of the amido fatty and other acids which are produced from the proteid. In some cases there will be a sufficiency of water in the lye for the production of the soap. If not, more water may be added after saponification has commenced.

Lower temperatures than those above herein specified may be used, but in that case the proteid matters are insufficiently acted on, and the process is prolonged with an inferior result.

As "cocoa-nut olein" either the oil as expressed from the nut may be employed, or the olein left after the removal of the stearin therefrom. The latter generally gives a drier and better result. The proteid matter which

we prefer to use is cocoa-nut cake, in fine powder. Cocoa-nut meal or other analogous meal containing an oil from which a soap soluble in sea-water can be produced may be 5 used but with much less certainty of result. Or, other nut- or cereal- or seed-meal may be employed which is relatively rich in proteid matters and which is substantially free from fatty acids, such for example as oatmeal, 10 bean-meal, maize-germ cake in powder and the like. When the proteid matter used is free from farina, it is usually advisable to add farina thereto, so as to produce a better lather. Generally from two to three parts 15 by weight of farina to one part of the proteid matter gives the best results.

We have found that the following proportions and method of procedure give excellent results, but it will be understood that we do 20 not limit ourselves thereto, since both may be varied within relatively wide limits. A lye is first made from 32 liters of concentrated solution of caustic soda and 9 liters of water. The "cocoa-nut olein", proteid, and 25 farina are then heated together, with stirring, to a temperature of about 105°C., for from 10 to 20 minutes, in the following proportions:—"cocoa-nut olein" 60 kilos, cocoa-nut oil cake, in powder 8 kilos, farina 24 30 kilos.

The above specified 41 liters of lye having a specific gravity of 1.465 are then gradually added with stirring, the temperature being maintained at between 80° and 100°C. When 35 the mass begins to thicken, there is added water 11 liters.

As soon as the saponification is completed, the mass may be transferred to a mold or frame to form bars, cakes, or the like, or it 40 may be allowed to cool and harden in the mixer, in which it can then be broken up sufficiently to allow it to be passed through a granulating sieve, preparatory to its being reduced to powder in a disintegrator after a 45 few hours drying. The product is preferred in a granulated, powdered or other like divided form as it is then more easily soluble in cold water and a lather is more easily produced.

A larger proportional quantity of "cocoa-nut olein" than that above specified may be used, in which case, the necessary increase in the quantity of lye must also be made. If a smaller quantity be used, the detergent will be too poor for laundry work, although it 55 may be useful for other purposes.

If the detergent is to be used for scouring purposes only, a larger quantity of lye may be employed.

Should a soft soap detergent be required, a 60 molecular proportion of potash lye is substituted for the whole or part of the soda lye.

We are aware that commercial olein and oatmeal and the like have already been acted on with strong lye in the cold in combination, 65 in the manufacture of detergent powders, but in that case the action on the proteid matter is very imperfect, and such proteid matter is not broken down with the separation of amino-fatty acids, and therefore such fatty 70 acids were not saponified as in our invention.

What we do claim as our invention and desire to secure by Letters Patent is:—

1. The process of producing a detergent for use with hard or salt waters, which consists in treating a vegetable proteid under heat with a sufficiency of strong alkali so as to break down the proteid with the disassociation of amino-fatty acids and saponifying the so separated amino fatty acids together 80 with cocoanut olein.

2. The process of producing a detergent for use with hard or salt waters, which consists in treating a vegetable proteid under heat with a sufficiency of strong alkali so as 85 to break down the proteid with the disassociation of amino-fatty acids and saponifying the so separated amino-fatty acids together with cocoanut olein, and finally adding a filling 90 material as specified.

In testimony whereof we have signed our names to this specification in the presence of two subscribing witnesses.

ROBERT MACPHERSON.  
WILLIAM EDWIN HEYS.

Witnesses:

H. D. JAMESON,  
F. L. RAND.